# EUROPEAN PATENT SPECIFICATION

(11) **EP 1 415 963 B1**
(45) Date of publication and mention of the grant of the patent: **08.03.2017**
(21) Application number: 03024880.1
(22) Date of filing: 31.10.2003
(51) Int. Cl.: C06D 5/06

(54) **Gas generating composition**
Gaserzeugende Zusammensetzung
Composition génératrice de gaz

(30) Priority: 31.10.2002 JP 2002317337; 21.10.2003 JP 2003360879; 24.10.2003 JP 2003364024
(43) Date of publication of application: 06.05.2004
(73) Proprietor: Daicel Chemical Industries, Ltd., Kita-ku, Osaka-shi Osaka 530-0001 (JP)
(72) Inventor: Yokoyama, Takushi, Himeji-shi Hyogo (JP); Watabiki, Mamoru, Himeji-shi Hyogo (JP); Wu, Jianzhou, Himeji-shi Hyogo (JP)
(74) Representative: Grünecker Patent- und Rechtsanwälte PartG mbB

(56) References cited:
- WO-A-01/34516
- WO-A-01/83274
- WO-A-99/46009
- DE-U- 29 821 541
- US-A- 5 035 757
- US-A- 5 460 668
- US-A- 6 143 102

## Description

### Technical Field

The present invention relates to a gas generating composition suitable for an air bag restraining system of automobiles and the like, a molded article thereof and an inflator for an air bag using the same.

### Background Art

As a gas generating agent for an air bag as a passenger-protecting system in automobiles, a composition using sodium azide has been conventionally used. However, a toxicity to human bodies [LD₅₀ (oral-rat) = 27 mg/kg] or hazard in handling of sodium azide has been regarded as a serious problem. Therefore, as safe non-azide based gas generating compositions, gas generating compositions containing various nitrogen-containing organic compounds have been developed to replace the above composition.

US-B 4,909,549 discloses a composition comprising hydrogen-containing tetrazole or triazole compounds and an oxygen-containing oxidizing agent. US-B 4,370,181 discloses a gas generating composition comprising a hydrogen-free bitetrazole metal salt and an oxygen-free oxidizing agent. US-B 4,369,079 discloses a gas generating composition comprising a hydrogen-free bitetrazole metal salt and an alkali metal nitrate, an alkali metal nitrite, an alkaline earth metal nitrate, an alkaline earth metal nitrite or a mixture thereof. US-B 5,542,999 discloses a gas generating agent comprising a fuel such as GZT, TAGN (triaminoguanidine nitrate), NG (nitroguanidine), NTO and the like, a basic copper nitrate, a catalyst for reducing toxic gases and a coolant. US-B 5,608,183 discloses a gas generating agent comprising a fuel such as guanidine nitrate, a basic copper nitrate and guar gum.

However, the above non-azide based gas generating composition forms residues (mist) after combustion, and thUS-B filter should be used to prevent the mist from flowing into an air bag. In this case, there is a method wherein the gas generating composition has a composition easily forming slag, after combustion, having a shape to be readily captured by the filter.

US-B 6,143,102 discloses that silica is added as a slag-forming agent to a composition comprising a fuel such as guanidine nitrate, a basic copper nitrate and a metal oxide such as alumina, to form excellent slag (clinker).

JP-A No. 10-502610 discloses that glass powder is added to a fuel such as a tetrazole compound and strontium nitrate, thereby lowering the combustion temperature, resulting in a reduction in NOx and CO and formation of solid slag.

US-B 5,104,466 (JP-A 5-70109) discloses that an alkali metal azide, pellets consisting of an oxidizing agent and grains consisting of a silica-containing material are used as a mixture to reduce mist.

WO-A-0183274 discloses a gas generator for a vehicle occupant protection system comprising: an elongated housing having a predetermined length and having a first send and a second end; a plurality of gas exit orifices spaced along the length of said housing; a propellant body contained within said housing, said propellant body having a length substantially coextensive with said housing; and an ignition body substantially coextensive with said propellant, said ignition body in physical contact with said propellant for substantially the length of said propellant and said ignition body having a burn rate at least twice that of said propellant body, wherein ignition of said ignition body essentially provides uniform ignition and combustion of said propellant body along the entire length thereof.

US-A-5035757 relates to a pyrotechnic, combustion filterable slag-particles forming gas generating mixture useful for inflating an automobile or aircraft safety crash bag, said pyrotechnic mixture comprising at least one material of each of the following functional groups of materials:
a. A fuel selected from the group of azole compounds consisting of triazole aminotetrazole, tetrazole, bitetrazole and metal salts of these compounds,
b. An oxygen containing oxidizer compound selected from the group consisting of alkali metal, alkaline earth metal, lanthanide and ammonium nitrates and perchlorates or from the group consisting of alkali metal and alkaline earth metal chlorates and peroxides,
c. A high temperature slag forming material selected from the group consisting of alkaline earth metal oxides, hydroxides, cabonates, and oxalates,
d. A low-temperature slag forming material which is sufficient in amount during combustion to cause the solid combustion particles to coalesce into easily filterable slag or clinkers but not so much as to make a low viscosity liquid, selected from the group consisting of silicon dioxide, boric oxide and vanadium pentoxide or from the group consisting of alkali metal silicates, borates, and carbonates or from the group consisting of naturally occurring clays and talcs.

WO-A-9946009 relates to a gas generant composition useful for inflating an automotive air bag passive restraint system comprising a mixture of: a high-nitrogen nonazide fuel selected from the class consisting of 1-, 3-, and 5-substituted amine salts of triazoles, and, 1- and 5-substituted amine salts of tetrazoles; a second fuel selected from the group consisting of hydrazodicarbonamide and azodicarbonamide; and phase stabilized ammonium nitrate.

### Disclosure of the Invention

Accordingly, a purpose of the present invention is to provide a novel gas generating composition forming slag more easily than the above compositions in the prior arts.

As means to solve the problem, the present invention provides a gas generating composition comprising the following components (a) to (d):
(a) 0.1 to 20% by mass of a glass powder having a softening point of 550°C or lower for forming a slag,
(b) 0.1 to 20% by mass of aluminum hydroxide,
(c) 30 to 60% by mass of an organic compound as fuel, and
(d) 30 to 60% by mass of a basic copper nitrate.

As still another means to solve the problem, the present invention provides a molded article in the form of a single-perforated cylinder or a perforated (porous) cylinder obtained from the above gas generating composition. The single-perforation or perforation may or may be a through-hole or a hollow.

As still further means to solve the problem, the present invention provides an inflator for an air bag using the gas generating composition or the molded article.

The gas generating composition of the present invention and a molded article thereof contain glass powder, by which combustion residues can be solidified to form a slag, thus preventing the combustion residues from being converted into mist and released to the outside of an inflator. This effect can further be improved by using glass powder in combination with aluminum hydroxide.

### Embodiments of the Invention

The glass powder used as component (a) in the present invention becomes molten upon combustion of the gas generating composition, and is immediately solidified as the temperature is decreased after combustion. In this process, the component (a) melts and solidifies combustion residues derived from other components, thereby trapping the residues to form a slag. Accordingly, the combustion residues are prevented from being converted into mist and released outside an inflator to flow in an air bag.

The glass powder is preferably an amorphous material consisting of a mixture of metal oxides and/or non-metal oxides, and the metal oxides are preferably those selected from silicon dioxide, sodium oxide, potassium oxide, calcium oxide, magnesium oxide, barium oxide, lead oxide, boron oxide, aluminum oxide and the like. The non-metal oxide is preferably selected from phosphorus oxide, tellurium oxide and bismuth oxide.

The glass powder is preferably one selected from the group consisting of quartz glass, 96% quartz glass, soda lime glass (windowpane, plate glass, bottle glass, glass for light bulb, etc.), lead glass (for electrical, optical and industrial art purposes), aluminoborosilicate glass, borosilicate glass (low expansion, low loss, tungsten sealing, etc.), aluminosilicate glass, phosphate glass, chalcogen glass, etc.

In particular, the softening point of such glass powder is 550°C or lower. With glass powder having a low softening point, the slag-forming effect is increased and mist is difficultly produced.

The glass powder having a low softening point includes, for example, phosphate glass (including P₂O₅ and one selected from CaO, B₂O₃, SiO₂, Al₂O₃, Fe₂O₃, MgO, Na₂O, K₂O and the like) or that represented by the following formula (I) :

xMnO-ySiO₂-zAl₂O₃ (I)

in which x, y and z are the mole number.

It is preferable that proportions of x, y and z of the formula (I) are 35 to 50 mole % of x, 30 to 60 mole % of y and 5 to 20 mole % of z, more preferably 40 to 45 mole % of x, 40 to 50 mole % of y and 10 to 15 mole % of z.

The particle diameter of the glass powder, in terms of 50% particle diameter, is preferably 10 to 300 µm, more preferably 10 to 100 µm, still more preferably 10 to 50 µm.

The content of the glass powder in the gas generating composition is 0.1 to 20% by mass, preferably 0.5 to 5% by mass. When the content of the glass powder is in the above range, the composition can preferably exhibit the slag-forming action without significantly lowering the efficiency of generation of gas.

Aluminum hydroxide used as component (b) is low in toxicity, has a high decomposition starting temperature, and shows a significantly endothermic reaction upon thermal decomposition, to form aluminum oxide and water. It follows that, by incorporation of aluminum hydroxide, the combustion temperature of the gas generating composition is decreased, and after combustion, the formed amount of toxic nitrogen oxides and carbon monoxide is decreased. Together with the glass powder as component (a), aluminum oxide formed by decomposition of aluminum hydroxide acts to form slag.

The content of aluminum hydroxide in the gas generating composition is 0.1 to 20% by mass, preferably 1 to 15% by mass. When the content of aluminum hydroxide is in the above-described range, the formed amount of toxic nitrogen oxides and carbon monoxide can be reduced as the combustion temperature is lowered, and when the gas generating composition is used in an inflator for an air bag, a burning rate necessary for expanding and developing an air bag in a predetermined time can also be assured.

The gas generating composition of the present invention can be in a four-component system consisting of (a) glass powder, (b) aluminum hydroxide, (c) an organic compound as fuel, and (d) an oxygen-containing oxidizing agent.

The organic compound as fuel of the component (c) is one or at least two selected from tetrazole compounds, guanidine compounds, triazine compounds and nitroamine compounds.

The tetrazole compounds include 5-aminotetrazole, bitetrazole ammonium, etc. The guanidine compounds include guanidine nitrate, mono-, di- or tri-aminoguanidine nitrate, nitroguanidine, etc. The triazine compounds include melamine, cyanuric acid, ammeline, ammelide, ammelande, etc.

The oxygen-containing oxidizing agent as component (d) a basic copper nitrate.

When the gas generating composition of the present invention is in a four-component system consisting of the components (a) to (d), the content of component (a) is 0.1 to 20% by mass, preferably 1 to 10% by mass, the content of component (b) is 0.1 to 20% by mass, preferably 1 to 15% by mass, the content of component (c) is 30 to 60% by mass, preferably 35 to 50% by mass, and the content of component (d) is 30 to 60% by mass, preferably 40 to 55% by mass.

A preferable example of the gas generating composition in a four-component system is a composition comprising (a) glass powder, (b) aluminum hydroxide, (c) guanidine nitrate and (d) a basic copper nitrate. In this case, the content of (a) glass powder is preferably 2 to 6% by mass, the content of (b) aluminum hydroxide is preferably 1 to 10% by mass, the content of (c) guanidine nitrate is preferably 30 to 60% by mass, and the content of (d) a basic copper nitrate is preferably 30 to 60% by mass.

Another preferable example of the gas generating composition in a four-component system is a composition comprising (a) glass powder, (b) aluminum hydroxide, (c) nitroguanidine and (d) a basic copper nitrate. In this case, the content of (a) glass powder is preferably 1 to 5% by mass, the content of (b) aluminum hydroxide is preferably 1 to 15% by mass, the content of (c) nitroguanidine is preferably 30 to 60% by mass, and the content of (d) a basic copper nitrate is preferably 30 to 60% by mass.

When the gas generating composition of the present invention is in a four-component system containing the components (a) to (d), or in a six-component system containing the components (a) to (d) and the component (f) of the additive and the component (g) of silicon dioxide, its molded article may, if poor in molding strength, collapse upon actual combustion and burn too acceleratedly to make control of combustion. Accordingly, the binder as component (e) is preferably added.

The binder as component (e) is one or at least two selected from carboxymethyl cellulose (CMC), sodium carboxymethylcellulose (CMCNa), potassium carboxymethylcellulose, carboxymethylcellulose ammonium, cellulose acetate, cellulose acetate butyrate (CAB), methyl cellulose (MC), ethyl cellulose (EC), hydroxyethyl cellulose (HEC), ethylhydroxyethyl cellulose (EHEC), hydroxypropyl cellulose (HPC), carboxymethylethyl cellulose (CMEC), fine crystalline cellulose, polyacrylamide, an aminated product of polyacrylamide, polyacryl hydrazide, a copolymer of acrylamide and a metal acrylate, a copolymer of polyacrylamide and a polyacrylic ester, polyvinyl alcohol, acrylic rubber, guar gum, starch and silicone. Among these, sodium carboyxmethylcellulose (CMCNa) and guar gum are preferable in view of stickiness, cost and ignitability of the binder.

The binder (e) is preferably contained in the gas generating composition in an amount of 1.0 to 5.0 mass %, more preferably 1.5 to 3.5 mass %, when it is combined with the component (b), not to lose a processability or moldability and make the combustion gas clear.

When the gas generating composition of the present invention is in a four-component system containing the components (a) to (d), or in a six-component system containing the components (a) to (d) and the component (e) of the binder and the component (g) of silicon dioxide, the additive as component (f) is added preferably for the purpose of assisting the actions of the components (a) and (b).

The additive as component (f) is one or at least two selected from metal oxides such as copper oxide, iron oxide, zinc oxide, cobalt oxide, manganese oxide, molybdenum oxide, nickel oxide, bismuth oxide, gallium oxide, silica and alumina, metal carbonates or basic metal carbonates such as cobalt carbonate, calcium carbonate, magnesium carbonate, a basic zinc carbonate and a basic copper carbonate, composite compounds of metal oxides or hydroxides such as Japanese acid clay, kaolin, talc, bentonite, diatomaceous earth and hydrotalcite, metal acid salts such as sodium silicate, mica molybdate, cobalt molybdate and ammonium molybdate, molybdenum disulfide, calcium stearate, silicon nitride and silicon carbide. These additives can reduce the burning temperature of the gas generating agent, regulate the burning rate and reduce the amount of toxic nitrogen oxides and carbon monoxide formed after combustion.

When the gas generating composition of the present invention is in a four-component system containing the components (a) to (d) or in a six-component system containing the components (a) to (d) and the component (e) of the binder and the component (f) of the additive, silicon dioxide as component (g) is preferably added for the purpose of improvement of ignition of the component (c). The ignition is greatly improved in particular with use of a guanidine compound for the component (c).

Silicon dioxide of the component (g) has a specific surface area of 100 to 500 m²/g, preferably 150 to 300 m²/g. The specific surface area is determined according to BET method.

Another preferable example of the gas generating composition in a five-component system is a composition comprising (a) glass powder, (b) aluminum hydroxide, (c) nitroguanidine, (d) a basic copper nitrate and (e) guar gum.

A still another preferable example of the gas generating composition in a five-component system is a composition comprising (a) glass powder, (b) aluminum hydroxide, (c) melamine, (d) a basic copper nitrate and (e) sodium carboxymethylcellulose or guar gum.

A still another preferable example of the gas generating composition in a five-component system is a composition comprising (a) glass powder, (b) aluminum hydroxide, (c) guanidine nitrate, (d) a basic copper nitrate and (e) sodium carboxymethylcellulose or guar gum.

A preferable example of the gas generating composition in not less than five-component system is a composition comprising (a) glass powder, (b) aluminum hydroxide, (c) a mixed fuel of two or three components selected from guanidine nitrate, nitroguanidine and melamine, (d) a basic copper nitrate and (e) sodium carboxymethylcellulose or guar gum.

A different, preferable embodiment is that including silicon dioxide of the component (g) in addition to the gas generating composition comprising the above shown (a) to (e).

The gas generating composition of the present invention can be molded in a desired shape, and formed into a molded article in the shape of a single-perforated cylinder, a perforated (porous) cylinder or pellets. These molded articles can be produced by a method in which the gas generating composition is mixed with water or an organic solvent and the mixture is extrusion-molded (molded articles in the shape of a single-perforated cylinder and a perforated (porous) cylinder) or by a compression-molding method using a pelletizer (molded article in the shape of pellets).

The gas generating composition of the present invention or the molded article obtained therefrom can be used in, for example, an inflator for an air bag of a driver side, and inflator for an air bag of a passenger side, an inflator for a air bag for a side collision, and inflator for an inflatable curtain, an inflator for a knee bolster, an inflator for an inflatable seat belt, an inflator for a tubular system and a gas generator for pretensioner in various vehicles.

Further, the inflator using the gas generating composition of the present invention or the molded article obtained therefrom may be a pyrotechnic type in which a gas is supplied only from a gas generating agent or a hybrid type in which a gas is supplied from both of a compressed gas such as argon and a gas generating agent.

Moreover, the gas generating composition of the present invention or the molded article obtained therefrom can also be used as an igniting agent called an enhancer (or a booster) for transferring energy of a detonator or a squib to a gas generating agent.

### Examples

The present invention is illustrated more specifically by referring to the following Examples, but the present invention is not limited thereto.

### Example 1 and Comparative Example 1

Gas generating compositions each having a formulation shown in Table 1 were produced, and each of the gas generating compositions was molded into 2 g of a strand. This strand was installed in a closed bomb having an inner capacity of 1 liter, and the inside of the bomb was purged with nitrogen. Further, the bomb was pressurized up to 6,860 kPa with nitrogen, and the strand was ignited by electrifying a nichrome wire and completely burned. After combustion, combustion residues were collected from the bomb and observed for their state with the naked eye.

In Table 1, GN is guanidine nitrate, BCN is a basic copper nitrate, CMCNa is sodium carboxymethylcellulose, and the glass powder has the following composition.

#C-490P (phosphate glass; softening point of about 400°C) (% by mass) : P₂O₅(54-56)/Al₂O₃ (9-11)/Na₂O (19-21)/K₂O (14-16)

**Table 1**

| | Formulation (formulation ratio: mass%) |
|---|---|
| Example 1 | # C-490P/Al(OH)₃/GN/BCN/CMCNa=2.0/9.8/41.9/43.8/2.5 |
| Comparative Example 1 | Al(OH)₃/GN/BCN/CMCNa=5/39.6/50.4/5 |

In Example 1, the strands after combustion maintained the shape thereof before combustion, but in Comparative Example 1, the strand was finely smashed.

## Claims

1. A gas generating composition comprising the following components (a) to (d):
(a) 0.1 to 20% by mass of a glass powder having a softening point of 550°C or lower for forming a slag,
(b) 0.1 to 20% by mass of aluminum hydroxide,
(c) 30 to 60% by mass of an organic compound as fuel and
(d) 30 to 60% by mass of a basic copper nitrate.

2. The gas generating composition as claimed in claim 1,
which further comprises at least one selected from the group consisting of the following components (e), (f) and (g), if required:
(e) a binder,
(f) an additive selected from a metal oxide and a metal carbonate and
(g) silicon dioxide having a specific surface area of 100 to 500 m²/g.

3. The gas generating composition as claimed in claim 2, wherein the content of the component (e) is 10% by mass or less, the content of the component (f) is 10% by mass or less and the content of the component (g) is 5% by mass or less.

4. The gas generating composition as claimed in any one of claims 1 to 3, wherein the glass powder as component (a) is an amorphous material consisting of a mixture of metal oxides and/or non-metal oxides.

5. The gas generating composition as claimed in claim 4, wherein the metal oxides are selected from the group consisting of silicon dioxide, sodium oxide, potassium oxide, calcium oxide, magnesium oxide, barium oxide, lead oxide, boron oxide and aluminum oxide.

6. The gas generating composition as claimed in any one of claims 1 to 5, wherein the glass powder as component (a) is selected from the group consisting of quartz glass, 96% quartz glass, soda lime glass, lead glass, aluminoborosilicate glass, borosilicate glass, aluminosilicate glass, phosphate glass and chalcogen glass.

7. The gas generating composition as claimed in any one of claims 1 to 5, wherein the glass powder as component (a) is represented by the following formula (I):
xMnO-ySiO₂-zAl₂O₃ (I)
in which x, y and z are the mole number.

8. The gas generating composition as claimed in claim 7, wherein proportions of x, y and z of the formula (I) are 35 to 50 mole% of x, 30 to 60 mole% of y and 5 to 20 mole% of z.

9. The gas generating composition as claimed in any one of claims 1 to 8, wherein the fuel as component (c) is at least one selected from the group consisting of tetrazole compounds, guanidine compounds, triazine compounds and nitroamine compounds.

10. The gas generating composition as claimed in any one of claims 2 to 9, wherein the binder as component (e) is at least one selected from the group consisting of carboxymethyl cellulose, sodium carboxymethylcellulose, potassium carboxymethylcellulose, carboxymethylcellulose ammonium, cellulose acetate, cellulose acetate butyrate, methyl cellulose, ethyl cellulose, hydroxyethyl cellulose, ethylhydroxyethyl cellulose, hydroxypropyl cellulose, carboxymethylethyl cellulose, fine crystalline cellulose, polyacrylamide, an aminated product of polyacrylamide, polyacryl hydrazide, a copolymer of an acrylamide and a metal acrylate, a copolymer of polyacrylamide and a polyacrylic ester, polyvinyl alcohol, acrylic rubber, guar gum, starch and silicone.

11. The gas generating composition as claimed in any one of claims 2 to 10, wherein the additive as component (f) is at least one selected from the group consisting of metal oxides including cupric oxide, iron oxide, zinc oxide, cobalt oxide, manganese oxide, molybdenum oxide, nickel oxide, bismuth oxide, gallium oxide, silica or alumina, metal hydroxides including cobalt hydroxide or iron hydroxide, metal carbonates or basic metal carbonates including cobalt carbonate, calcium carbonate, magnesium carbonate, a basic zinc carbonate or a basic copper carbonate, composite compounds of metal oxides or metal hydroxides including Japanese acid clay, kaolin, talc, bentonite, diatomaceous earth or hydrotalcite, metal acid salts including sodium silicate, mica molybdate, cobalt molybdate or ammonium molybdate, silicone, molybdenum disulfide, calcium stearate, silicon nitride and silicon carbide.

12. The gas generating composition as claimed in any one of claims 2 to 11, wherein the binder (e) is contained in an amount of 1.0 to 5.0 mass%.

13. The gas generating composition as claimed in any one of claims 1 to 12, wherein the organic compound (c) is guanidine nitrate.

14. A molded article of the gas generating composition being in the shape of a single perforated cylinder or a perforated cylinder, obtained by extrusion-molding the gas generating composition as defined in any one of claims 1 to 13.

15. An inflator for air bag, using the gas generating composition as defined in any one of claims 1 to 13 or using the molded article of the gas generating composition as defined in claim 14.

## Patentansprüche

1. Gaserzeugende Zusammensetzung, umfassend die folgenden Komponenten (a) bis (d):
(a) 0,1 bis 20 Massen% eines Glaspulvers mit einem Erweichungspunkt von 550 °C oder niedriger zum Bilden einer Schlacke,
(b) 0,1 bis 20 Massen% Aluminiumhydroxid,
(c) 30 bis 60 Massen% einer organischen Verbindung als Treibstoff und
(d) 30 bis 60 Massen% eines basischen Kupfernitrats.

2. Gaserzeugende Zusammensetzung wie in Anspruch 1 beansprucht,
welche außerdem wenigstens eine Komponente, ausgewählt aus der Gruppe bestehend aus den folgenden Komponenten (e), (f) und (g), umfasst, falls erforderlich:
(e) ein Bindemittel,
(f) ein Additiv, ausgewählt aus einem Metalloxid und einem Metallcarbonat, und
(g) Siliciumdioxid mit einer spezifischen Oberfläche von 100 bis 500 m²/g.

3. Gaserzeugende Zusammensetzung wie in Anspruch 2 beansprucht, wobei der Gehalt der Komponente (e) 10 Massen% oder weniger beträgt, der Gehalt der Komponente (f) 10 Massen% oder weniger beträgt, und der Gehalt der Komponente (g) 5 Massen% oder weniger beträgt.

4. Gaserzeugende Zusammensetzung wie in einem der Ansprüche 1 bis 3 beansprucht, wobei das Glaspulver als Komponente (a) ein amorphes Material ist, das aus einer Mischung aus Metalloxiden und/oder Nichtmetalloxiden besteht.

5. Gaserzeugende Zusammensetzung wie in Anspruch 4 beansprucht, wobei die Metalloxide ausgewählt sind aus der Gruppe bestehend aus Siliciumdioxid, Natriumoxid, Kaliumoxid, Calciumoxid, Magnesiumoxid, Bariumoxid, Bleioxid, Boroxid und Aluminiumoxid.

6. Gaserzeugende Zusammensetzung wie in einem der Ansprüche 1 bis 5 beansprucht, wobei das Glaspulver als Komponente (a) ausgewählt ist aus der Gruppe bestehend aus Quarzglas, 96 %igem Quarzglas, Kalknatronglas, Bleiglas, Aluminiumborosilicatglas, Borosilicatglas, Aluminiumsilicatglas, Phosphatglas und Chalcogenglas.

7. Gaserzeugende Zusammensetzung wie in einem der Ansprüche 1 bis 5 beansprucht, wobei das Glaspulver als Komponente (a) durch die folgende Formel (I) wiedergegeben ist:
xMnO-ySiO₂-zAl₂O₃ (I)
in welcher x, y und z die Molzahl sind.

8. Gaserzeugende Zusammensetzung wie in Anspruch 7 beansprucht, wobei die Anteile von x, y und z der Formel (I) 35 bis 50 Mol% x, 30 bis 60 Mol% y und 5 bis 20 Mol% z sind.

9. Gaserzeugende Zusammensetzung wie in einem der Ansprüche 1 bis 8 beansprucht, wobei der Treibstoff als Komponente (c) wenigstens eine Verbindung, ausgewählt aus der Gruppe bestehend aus Tetrazolverbindungen, Guanidinverbindungen, Triazinverbindungen und Nitroaminverbindungen, ist.

10. Gaserzeugende Zusammensetzung wie in einem der Ansprüche 2 bis 9 beansprucht, wobei das Bindemittel als Komponente (e) wenigstens ein Bindemittel, ausgewählt aus der Gruppe bestehend aus Carboxymethylcellulose, Natriumcarboxymethylcellulose, Kaliumcarboxymethylcellulose, Carboxymethylcellulose-ammonium, Celluloseacetat, Celluloseacetatbutyrat, Methylcellulose, Ethylcellulose, Hydroxyethylcellulose, Ethylhydroxyethylcellulose, Hydroxypropylcellulose, Carboxymethylethylcellulose, feinkristalliner Cellulose, Polyacrylamid, einem aminierten Produkt von Polyacrylamid, Polyacrylhydrazid, einem Copolymer von einem Acrylamid und einem Metallacrylat, einem Copolymer von Polyacrylamid und einem Polyacrylester, Polyvinylalkohol, Acrylkautschuk, Guargummi, Stärke und Silicon, ist.

11. Gaserzeugende Zusammensetzung wie in einem der Ansprüche 2 bis 10 beansprucht, wobei das Additiv als Komponente (f) wenigstens ein Additiv, ausgewählt aus der Gruppe bestehend aus Metalloxiden einschließlich Kupfer(II)-oxid, Eisenoxid, Zinkoxid, Cobaltoxid, Manganoxid, Molybdänoxid, Nickeloxid, Wismutoxid, Galliumoxid, Siliciumdioxid oder Aluminiumoxid, Metallhydroxiden einschließlich Cobalthydroxid oder Eisenhydroxid, Metallcarbonaten oder basischen Metallcarbonaten einschließlich Cobaltcarbonat, Calciumcarbonat, Magnesiumcarbonat, eines basischen Zinkcarbonats oder eines basischen Kupfercarbonats, Verbundverbindungen von Metalloxiden oder Metallhydroxiden einschließlich japanischer saurer Tonerde, Kaolin, Talk, Bentonit, Diatomeenerde oder Hydrotalcit, Metallsäuresalzen einschließlich Natriumsilicat, Glimmermolybdat, Cobaltmolybdat oder Ammoniummolybdat, Silicon, Molybdändisulfid, Calciumstearat, Siliciumnitrid und Siliciumcarbid, ist.

12. Gaserzeugende Zusammensetzung wie in einem der Ansprüche 2 bis 11 beansprucht, wobei das Bindemittel (e) in einer Menge von 1,0 bis 5,0 Massen% enthalten ist.

13. Gaserzeugende Zusammensetzung wie in einem der Ansprüche 1 bis 12 beansprucht, wobei die organische Verbindung (c) Guanidinnitrat ist.

14. Formteil aus der gaserzeugenden Zusammensetzung in Form eines einfach perforierten Zylinders oder eines perforierten Zylinders, erhalten durch Extrusionsformen der gaserzeugenden Zusammensetzung wie in einem der Ansprüche 1 bis 13 definiert.

15. Gasgenerator für einen Airbag, der die gaserzeugende Zusammensetzung, wie in einem der Ansprüche 1 bis 13 definiert, verwendet oder das Formteil aus der gaserzeugenden Zusammensetzung, wie in Anspruch 14 definiert, verwendet.

## Revendications

1. Composition génératrice de gaz comprenant les composants (a) à (d) suivants :
(a) 0,1 à 20 % en masse d'une poudre de verre ayant un point de ramollissement de 550 °C ou moins pour former un laitier,
(b) 0,1 à 20 % en masse d'hydroxyde d'aluminium,
(c) 30 à 60 % en masse d'un composé organique comme combustible et
(d) 30 à 60 % en masse d'un nitrate de cuivre basique.

2. Composition génératrice de gaz ainsi que revendiquée dans la revendication 1,
qui comprend en outre au moins un composant choisi dans le groupe constitué des composants suivants (e), (f) et (g), si nécessaire :
(e) un liant,
(f) un additif choisi parmi un oxyde métallique et un carbonate métallique et
(g) du dioxyde de silicium ayant une surface spécifique de 100 à 500 m²/g.

3. Composition génératrice de gaz telle que revendiquée dans la revendication 2, dans laquelle la teneur du composant (e) est de 10 % en masse ou moins, la teneur du composant (f) est de 10 % en masse ou moins et la teneur du composant (g) est de 5 % en masse ou moins.

4. Composition génératrice de gaz telle que revendiquée dans l'une quelconque des revendications 1 à 3, dans laquelle la poudre de verre en tant que composant (a) est un matériau amorphe constitué d'un mélange d'oxydes métalliques et/ou d'oxydes non métalliques.

5. Composition génératrice de gaz telle que revendiquée dans la revendication 4, dans laquelle les oxydes métalliques sont choisis dans le groupe constitué de dioxyde de silicium, oxyde de sodium, oxyde de potassium, oxyde de calcium, oxyde de magnésium, oxyde de baryum, oxyde de plomb, oxyde de bore et oxyde d'aluminium.

6. Composition génératrice de gaz telle que revendiquée dans l'une quelconque des revendications 1 à 5, dans laquelle la poudre de verre en tant que composant (a) est choisie dans le groupe constitué de verre de quartz, verre de quartz à 96 %, verre sodocalcique, verre au plomb, verre aluminoborosilicaté, verre borosilicaté, verre aluminosilicaté, verre phosphaté, verre de chalcogénure.

7. Composition génératrice de gaz telle que revendiquée dans l'une quelconque des revendications 1 à 5, dans laquelle la poudre de verre en tant que composant (a) est représentée par la formule suivante (I) :
xMnO-ySiO₂-zAl₂O₃ (I)
dans laquelle x, y et z sont le nombre de moles.

8. Composition génératrice de gaz telle que revendiquée dans la revendication 7, dans laquelle les proportions de x, y et z dans la formule (I) sont de 35 à 50 % en mole de x, 30 à 60 % en mole de y et 5 à 20 % de mole de z.

9. Composition génératrice de gaz telle que revendiquée dans l'une quelconque des revendications 1 à 8, dans laquelle le combustible en tant que composant (c) est au moins un composé choisi dans le groupe constitué de composés tétrazole, composés guanidine, composés triazine et composés nitroamine.

10. Composition génératrice de gaz telle que revendiquée dans l'une quelconque des revendications 2 à 9, dans laquelle le liant en tant que composant (e) est l'un au moins choisi dans le groupe constitué de carboxyméthylcellulose, carboxyméthycellulose sodique, carboxyméthylcellulose potassique, carboxyméthylcellulose d'ammonium, acétate de cellulose, acétate butyrate de cellulose, méthyl-cellulose, éthylcellulose, hydroxyéthylcellulose, éthylhydroxyéthylcellulose, hydroxypropylcellulose, carboxyméthyléthylcellulose, cellulose cristalline fine, polyacrylamide, un produit aminé de polyacrylamide, polyacrylhydrazide, un copolymère d'un acrylamide et d'un acrylate de métal, un copolymère de polyacrylamide et d'un ester polyacrylique, alcool polyvinylique, caoutchouc acrylique, gomme de guar, amidon et silicone.

11. Composition génératrice de gaz telle que revendiquée dans l'une quelconque des revendications 2 à 10, dans laquelle l'additif en tant que composant (f) est l'un au moins choisi dans le groupe constitué d'oxydes métalliques notamment oxyde cuprique, oxyde de fer, oxyde de zinc, oxyde de cobalt, oxyde de manganèse, oxyde de molybdène, oxyde de nickel, oxyde de bismuth, oxyde de gallium, silice ou alumine, hydroxydes métalliques notamment hydroxyde de cobalt ou hydroxyde de fer, carbonates métalliques ou carbonates métalliques basiques notamment carbonate de cobalt, carbonate de calcium, carbonate de magnésium, un carbonate de zinc basique ou un carbonate de cuivre basique, composés composites d'oxydes métalliques ou d'hydroxydes métalliques notamment argile acide du Japon, kaolin, talc, bentonite, terre de diatomées ou hydrotalcite, des sels d'acides métalliques notamment silicate de sodium, molybdate de mica, molybdate de cobalt ou molybdate d'ammonium, silicone, disulfure de molybdène, stéarate de calcium, nitrure de silicium et carbure de silicium.

12. Composition génératrice de gaz telle que revendiquée dans l'une quelconque des revendications 2 à 11, dans laquelle le liant (e) est présent en une quantité de 1,0 à 5,0 % en masse.

13. Composition génératrice de gaz telle que revendiquée dans l'une quelconque des revendications 1 à 12, dans laquelle le composé organique (c) est le nitrate de guanidine.

14. Article moulé à partir de la composition génératrice de gaz sous la forme d'un cylindre mono-perforé ou d'un cylindre perforé, obtenu par moulage par extrusion de la composition génératrice de gaz telle que définie dans l'une quelconque des revendications 1 à 13.

15. Gonfleur de coussin gonflable, utilisant la composition génératrice de gaz telle que définie dans l'une quelconque des revendications 1 à 13 ou utilisant l'article moulé à partir de la composition génératrice de gaz tel que défini dans la revendication 14.
